

Patented Oct. 20, 1925.

1,558,265

## UNITED STATES PATENT OFFICE.

ISIDORE OCTAVE EMILE LAMS, OF TUBIZE, BELGIUM, ASSIGNOR TO FABRIQUE DE SOIE ARTIFICIELLE DE TUBIZE, SOCIÉTÉ ANONYME, OF BRUSSELS, BELGIUM.

### PROCESS OF MANUFACTURING ARTIFICIAL-SILK THREADS FROM VISCOSE.

No Drawing.

Application filed January 18, 1923. Serial No. 613,541.

To all whom it may concern:

Be it known that I, ISIDORE OCTAVE EMILE LAMS, a subject of the King of the Belgians, residing at Tubize, in the Kingdom of Belgium, have invented certain new and useful Improvements in the Process of Manufacturing Artificial-Silk Threads from Viscose, of which the following is a specification.

My invention relates to a process of manufacturing artificial silk threads from viscose.

One object of my invention is to produce a thread of cellulose xanthate which will be more extensible than the threads hitherto obtained so that it can be drawn out into a very thin thread before being precipitated into a thread of cellulose hydrate. And a further object of my invention is to improve the brilliancy and suppleness of the thread thus obtained.

With these objects in view my invention consists in making use of a special coagulating bath composed of ammonium formate at the minimum required concentration to neutralize the free soda which is present in the viscose solution and of sodium formate at the minimum required concentration to secure coagulation.

Experiences have shown that the following proportions secure the best results:

Ammonium formate 13 to 15 parts in weight and sodium formate 13 to 18 parts in weight, these substances being dissolved in the necessary quantity of water to obtain 35 100 parts in weight of the coagulating bath.

When using such a coagulating bath, a transparent thread having a clear yellow appearance is obtained, which can be very easily drawn out into a very thin thread and

which possess a coefficient of drawing of 40 98%, that is to say that a length of 1 m. of the elementary thread or filaments issuing from the spinning orifice can be drawn or stretched so as to present an increase of 45 length of 98 cm. before breaking.

In carrying my invention into practice the viscose solution is projected as usually through fine orifices into the above stated coagulating bath; the thread is drawn out according to the well known method and is 50 finally precipitated in the form of a thread of cellulose hydrate by any well known method for instance by aid of an acid solution of weak concentration. It is however advisable to make this decomposition rapidly so as to avoid any possible disturbance in working resulting from the sticking or gluing of the threads to each other.

What I claim is:

1. In the process of manufacturing artificial silk threads from viscose, the steps which comprise subjecting viscose threads to the action of an aqueous solution containing 13 to 15% of ammonium formate and 13 to 18% of sodium formate, drawing the 65 threads while so coagulated, and then converting them into cellulose hydrate.

2. As a new composition of matter, an aqueous solution of 13 to 15% of ammonium formate and 13 to 18% of sodium formate, 70 the said composition having coagulating properties whereby viscose threads are converted into extensible cellulose xanthate threads.

In testimony whereof I have affixed my 75 signature.

ISIDORE OCTAVE EMILE LAMS.